# EUROPEAN PATENT SPECIFICATION

(11) **EP 1 195 426 B1**
(45) Date of publication and mention of the grant of the patent: **15.08.2007**
(21) Application number: 01203645.5
(22) Date of filing: 24.09.2001
(51) Int. Cl.: C10M 163/00

(54) **Lubricating oil composition for gas-fuelled engines**
Schmierölzusammensetzung für flüssiggasbetriebene Brennkraftmaschine
Composition d'huile lubrifiante pour moteur alimenté en gaz liquéfié

(30) Priority: 05.10.2000 EP 00121752
(43) Date of publication of application: 10.04.2002
(73) Proprietor: Infineum International Limited, Abingdon, Oxon OX13 6BB (GB)
(72) Inventor: Garner, Mr. Terence, Didcot, Oxfordshire OX11 7SU (GB); Chambard, Mr. Laurent, Stanford in the Vale, Oxfordshire SN7 8NQ (GB); Dunn, Mr. Adrian, Faringdon, Oxfordshire SN7 7RN (GB)
(74) Representative: Lewis, Pauline Therese

(56) References cited:
- WO-A-94/28095
- WO-A-97/46645
- US-A- 5 726 133
- US-A- 5 792 735
- US-A- 5 906 969
- US-A- 6 034 039

## Description

This invention relates to gas-fuelled engine lubrication.

Gas-fuelled engines, sometimes referred to as gas-fired engines or merely gas engines, are known and may be used in the oil and gas industry, for example, to drive pumping stations of natural gas pipelines, blowers and generators in purification plants and on gas tankers, to compress natural gas at well heads and along pipe lines and to produce electric power in fit-for-purpose plants. Their design may be two- or four-stroke, spark-ignited or compression-ignited, though four-stroke compression-ignited designs constitute a large percentage. Natural gas constitutes a typical fuel.

Problems in their lubrication are firstly, that the lubricant is subjected to sustained high temperatures leading to its oxidation, and secondly, that the engines emit relatively high quantities of oxides of nitrogen, leading to nitration of the lubricant. These problems reduce the working life of the lubricant.

US-A-5 726 133 describes a way of meeting the above problems by using, in a natural gas engine oil, an additive mixture comprising a mixture of detergents comprising at least one first alkali or alkaline earth metal salt or mixture thereof of TBN of 250 and less, and at least one second alkali or alkaline earth metal salt or mixture thereof which is more neutral than the first salt.

EP-A-0 860 495 describes a lubricating oil composition stated to be excellent for NOx oxidation resistance and thermal oxidation resistance and suitable as a long-life engine oil for gas engine heat pumps. The composition includes a metal salicylate having a TBN of from 100 to 195, and optionally includes a metal phenate having a TBN of from 100 to 300.

There is, however, a desire to further improve the lubricant performance in the above respects, for example to enable the interval between lubricant changes to be extended.

The present invention meets this desire, as evidenced by and in the examples hereof, by using, as a first detergent, a salicylate having a TBN of 95 or less and a second detergent having a TBN of greater than 250.

US 5,906,969 discloses lubricating oils for improving the fuel economy of internal combustion engines.

Accordingly, a first aspect of the present invention is a gas-fuelled engine lubricating oil composition having a TBN in the range of 2 to 20 comprising:
(A) an oil of lubricating viscosity, in a major amount; and added thereto, in respective minor amounts:
(B) one or more metal hydrocarbyl-substituted salicylate detergents having a TBN of 95 or less, preferably 85 or less, more preferably 75 or less;
(C) one or more calcium salicylate, phenate or complex detergents having a TBN of greater than 250, preferably greater than 265, more preferably greater than 275;
(D) one or more dispersants, such as an ashless dispersant; and
(E) preferably one or more anti-wear additives.

A second aspect of the present invention is a method of lubricating a gas-fuelled internal combustion engine, the method comprising operating the engine and lubricating it with the composition defined above according to the first aspect of the invention.

A third aspect of the present invention is a method for enhancing the resistance of a gas-fuelled lubricating oil composition to oxidation and nitration, the method comprising the step of adding additives (B) to (E) as defined in the first aspect of the invention to the gas-fuelled lubricating oil composition.

"Major amount" means in excess of 50 mass % of the composition.

"Minor amount" means less than 50 mass % of the composition, both in respect of the stated additive and in respect of the total mass % of all the additives present in composition, reckoned as active ingredient of the additive or additives.

"Comprises or comprising" or cognate words is taken to specify the presence of stated features, steps, integers or components, but does not preclude the presence or addition of one or more other features, steps, integer components or groups thereof.

"TBN" (Total Base Number) is as measured by ASTM D2896.

Unless otherwise started, all proportions are expressed as mass % active ingredient, i.e. as if solvent or diluent or other inert material were absent.

The features of the invention will now be discussed in more detail below.

### Lubricating Oil Composition

Preferably, the TBN of the lubricant composition is in the range of from 2 to 20, such as from 2.5 to 20, preferably from 6.5 to 20, more preferably from 6.5 to 15.

### (A) Oil of Lubricating Viscosity

The oil of lubricating viscosity (sometimes referred to as lubricating oil) may be any oil suitable for the lubrication of a gas-fuelled engine. The lubricating oil may suitably be an animal, a vegetable or a mineral oil. Suitably the lubricating oil is a petroleum-derived lubricating oil, such as a naphthenic base, paraffinic base or mixed base oil. Alternatively, the lubricating oil may be a synthetic lubricating oil. Suitable synthetic lubricating oils include synthetic ester lubricating oils, which oils include diesters such as di-octyl adipate, di-octyl sebacate and tridecyl adipate, or polymeric hydrocarbon lubricating oils, for example liquid polyisobutene and poly-alpha olefins. Commonly, a mineral oil is employed. The lubricating oil may generally comprise greater than 60, typically greater than 70, mass % of the composition, and typically have a kinematic viscosity at 100°C of from 2 to 40, for example for 3 to 15, mm²s⁻¹ and a viscosity index of from 80 to 100, for example from 90 to 95.

Another class of lubricating oils is hydrocracked oils, where the refining process further breaks down the middle and heavy distillate fractions in the presence of hydrogen at high temperatures and moderate pressures. Hydrocracked oils typically have a kinematic viscosity at 100°C of from 2 to 40, for example from 3 to 15, mm²s⁻¹ and a viscosity index typically in the range of from 100 to 110, for example from 105 to 108.

The oil may include 'brightstock' which refers to base oils which are solvent-extracted, de-asphalted products from vacuum residuum generally having a kinematic viscosity at 100°C of from 28 to 36 mm²s⁻¹ and are typically used in a proportion of less than 30, preferably less than 20, more preferably less than 15, most preferably less than 10, such as less than 5, mass %, based on the mass of the composition.

### (B) Salicylate Detergent

A detergent is an additive that reduces formation of piston deposits, for example high-temperature varnish and lacquer deposits, in engines; it has acid-neutralising properties and is capable of keeping finely divided solids in suspension. It is based on metal "soaps", that is metal salts of acidic organic compounds, sometimes referred to as surfactants, which, in respect of (B), is salicylic acid.

The detergent comprises a polar head with a long hydrophobic tail, the polar head comprises a metal salt of the salicylic acid. Large amounts of a metal base are included by reacting an excess of a metal compound, such as an oxide or hydroxide, with an acidic gas such as carbon dioxide to give an overbased detergent which comprises neutralised detergent as the outer layer of a metal base (e.g. carbonate) micelle.

The metal may be an alkali or alkaline earth metal, e.g., sodium, potassium, lithium, calcium, and magnesium. Calcium is preferred.

Surfactants for the surfactant system of the overbased metal detergents contain at least one hydrocarbyl group, for example, as a substituent on an aromatic ring. The term "hydrocarbyl" as used herein means that the group concerned is primarily composed of hydrogen and carbon atoms and is bonded to the remainder of the molecule via a carbon atom, but does not exclude the presence of other atoms or groups in a proportion insufficient to detract from the substantially hydrocarbon characteristics of the group. Advantageously, hydrocarbyl groups in surfactants for use in accordance with the invention are aliphatic groups, preferably alkyl or alkylene groups, especially alkyl groups, which may be linear or branched. The total number of carbon atoms in the surfactants should be at least sufficient to impact the desired oil-solubility.

The salicylates may be non-sulfurized or sulfurized, and may be chemically modified and/or contain additional substitutents. Processes for sulfurizing a hydrocarbyl-substituted salicylic acid are well known to those skilled in the art. Salicylic acids are typically prepared by the carboxylation, by the Kolbe-Schmitt process, of phenoxides, and in that case, will generally be obtained, normally in a diluent, in admixture with uncarboxylated phenol.

Preferred substituents in oil-soluble salicylic acids from which the salicylates may be derived are alkyl substituents. In alkyl-substituted salicylic acids, the alkyl groups advantageously contain 5 to 100, preferably 9 to 30, especially 14 to 20, carbon atoms. Where there are more than one alkyl groups, the average number of carbon atoms in all of the alkyl groups is preferably at least 9 to ensure adequate oil-solubility.

The gas-fuelled engine lubricating oil composition preferably includes only one metal hydrocarbyl-substituted salicylate detergent having a TBN of 95 or less, component (B).

The salicylate may be used in a proportion in the range of 0.5 to 30, preferably 2 to 15 or to 20, mass % based on the mass of the lubricating oil composition.

### (C) Calcium Salicylate, Phenate or Complex Detergents having a TBN greater than 250

Component (C) is one or more calcium salicylate, phenate or complex detergents having a TBN of greater than 250.

Complex detergents comprise an overbased mixture of at least two calcium surfactants, such as a calcium alkyl phenate and a calcium alkyl salicylate. Such a complex detergent is a hybrid material in which the surfactant groups, e.g. phenate and salicylate, are incorporated during the overbasing process.
Examples of complex detergents are described in the art.

Another example of a detergent that may be used comprises a sulfurized and then overbased mixture of a calcium alkyl phenate and a calcium alkyl salicylate such as described in EP-A-750,659, for example as:
a detergent-dispersant additive for lubricating oil of the sulfurised and superalkalinised, alkaline earth alkylsalicylate-alkylphenate type, characterised in that:
   (a) the alkyl substituents of the said alkylsalicylate-alkylphenate are in a proportion of at least 35 wt.% and at most 85 wt.% of linear alkyl in which the number of carbon atoms is between 12 and 40, preferably between 18 and 30 carbon atoms, with a maximum of 65 wt.% of branched alkyl in which the number of carbon atoms is between 9 and 24 and preferably 12 carbon atoms;
   (b) the proportion of alkylsalicylate in the alkylsalicylate-alkylphenate mixture is at least 22 mole % and preferably at least 25 mole %, and
   (c) the molar proportion of alkaline in the alkylsalicylate-alkylphenate as a whole is between 1.0 and 3.5.

Preferably, the calcium detergents (C) have a TBN in the range of 250 to 500, more preferably 260 to 400.

### (D) Dispersants

A dispersant is an additive for a lubricating composition whose primary function is to hold solid and liquid contaminants in suspension, thereby passivating them and reducing engine deposits at the same time as reducing sludge depositions. Thus, for example, a dispersant maintains in suspension oil-insoluble substances that result from oxidation during use of the lubricating oil, thus preventing sludge flocculation and precipitation or deposition on metal parts of the engine.

A noteworthy class of dispersants are "ashless", meaning a non-metallic organic material that forms substantially no ash on combustion, in contrast to metal-containing, hence ash-forming, materials. Ashless dispersants comprise a long chain hydrocarbon with a polar head, the polarity being derived from inclusion of, e.g. an O, P or N atom. The hydrocarbon is an oleophilic group that confers oil-solubility, having for example 40 to 500 carbon atoms. Thus, ashless dispersants may comprise an oil-soluble polymeric hydrocarbon backbone having functional groups that are capable of associating with particles to be dispersed.

Examples of ashless dispersants are succinimides, e.g. polyisobutene succinic anhydride; and polyamine condensation products that may be borated or unborated.

### (E) Antiwear Additive

The antiwear additives may be metallic or non-metallic, preferably the former.

Dihydrocarbly dithiophosphate metal salts are examples of the anti-wear additives used in the present invention. The metal in the dihydrocarbyl dithiophosphate metal may be an alkali or alkaline earth metal, or aluminium, lead, tin, molybdenum, manganese, nickel or copper. Zinc salts are preferred, preferably in the range of 0.1 to 1.5, preferably 0.5 to 1.3, mass %, based upon the total mass of the lubricating oil composition. They may be prepared in accordance with known techniques by firstly forming a dihydrocarbyl dithiophosphoric acid (DDPA), usually by reaction of one or more alcohols or a phenol with P₂S₅ and then neutralizing the formed DDPA with a zinc compound. For example, a dithiophosphoric acid may be made by reacting mixtures of primary and secondary alcohols. Alternatively, multiple dithiophosphoric acids can be prepared comprising both hydrocarbyl groups that are entirely secondary and hydrocarbyl groups that are entirely primary. To make the zinc salt, any basic or neutral zinc compound may be used but the oxides, hydroxides and carbonates are most generally employed. Commercial additives frequently contain an excess of zinc due to use of an excess of the basic zinc compound in the neutralisation reaction.

The preferred zinc dihydrocarbyl dithiophosphates are oil-soluble salts of dihydrocarbyl dithiophosphoric acids and may be represented by the following formula:

[(RO) (R'O) P(S)S]₂ Zn

where R and R' may be the same or different hydrocarbyl radicals containing from 1 to 18, preferably 2 to 12, carbon atoms and including radicals such as alkyl, alkenyl, aryl, arylalkyl, alkaryl and cycloaliphatic radicals. Particularly preferred as R and R' groups are alkyl groups of 2 to 8 carbon atoms. Thus, the radicals may, for example, be ethyl, n-propyl, I-propyl, n-butyl, I-butyl, sec-butyl, amyl, n-hexyl, I-hexyl, n-octyl, decyl, dodecyl, octadecyl, 2-ethylehexyl, phenyl, butylphenyl, cyclohexyl, methylcyclopentyl, propenyl, butenyl. In order to obtain oil-solubility, the total number of carbon atoms (i.e. in R and R¹) in the dithiophoshoric acid will generally be 5 or greater. The zinc dihydrocarbyl dithiophosphate can therefore comprise zinc dialkyl dithiophosphates.

The composition of the present invention may, optionally, have further added there-to in a minor amount (F) one or more antioxidants as discussed in further detail below.

### (F) Anti-oxidants

As stated these may be amines or phenolic. As examples of amines there may be mentioned secondary aromatic amines such as diarylamines, for example diphenylamines wherein each phenyl group is alkyl-substituted with an alkyl group having 4 to 9 carbon atoms. As examples of anti-oxidants there may be mentioned hindered phenols, including mono-phenols and bis-phenols.

Preferably, the anti-oxidant, if present, is provided in the composition in an amount of up to 3 mass %.

Other additives such as pour point depressants, anti-foamants, and/or demulsifiers may be provided, if necessary.

It may be desirable, although not essential, to prepare one or more additive packages or concentrates comprising the additives, whereby additives (B) to (E), and (F) if provided, can be added simultaneously to the base oil to form the lubricating oil composition. Dissolution of the additive package(s) into the lubricating oil may be facilitated by solvents and by mixing accompanied with mild heating, but this is not essential. The additive package(s) will typically be formulated to contain the additive(s) in proper amounts to provide the desired concentration, and/or to carry out the intended function in the final formulation when the additive package(s) is/are combined with a predetermined amount of base lubricant. Thus, additives (B) to (E), and (F) if provided, in accordance with the present invention, may be admixed with small amounts of base oil or other compatible solvents together with other desirable additives to form additive packages containing active ingredients in an amount, based on the additive package, of, for example, from 2.5 to 90, preferably from 5 to 75, most preferably from 8 to 60, mass % of additives in the appropriate proportions, the remainder being base oil.

The final formulations may typically contain about 5 to 40 mass % of the additive packages(s), the remainder being base oil.

The term 'active ingredient' (a.i.) as used herein refers to the additive material that is not diluent.

The terms 'oil-soluble' or 'oil-dispersable' as used herein do not necessarily indicate that the compounds or additives are soluble, dissolvable, miscible or capable of being suspended in the oil in all proportions. These do mean, however, that they are, for instance, soluble or stably dispersible in oil to an extent sufficient to exert their intended effect in the environment in which the oil is employed.
Moreover, the additional incorporation of other additives may also permit incorporation of higher levels of a particular additive, if desired.

The lubricant compositions of this invention comprise defined individual (i.e. separate) components that may or may not remain the same chemically before and after mixing.

### Examples

The present invention is illustrated by, but in no way limited to, the following examples.

### Examples 1 & 2

Gas-fuelled engine lubricating oil compositions of the invention were prepared by blending methods known in the art. Their compositions were as follows:

| COMPONENTS | | Example 1 | Example 2 |
|---|---|---|---|
| (B) | Ca salicylate, TBN 65 | 3.46 | 3.85 |
| (C) | Ca salicylate, TBN 281 | 0.35 | 0.39 |
| (D) | Borated succinimide dispersant | 3.41 | 3.80 |
| | Unborated succinimide dispersant | 2.58 | 2.88 |
| (E) | ZDDP anti-wear additive | 0.26 | 0.29 |
| (F) | Diphenylamine anti-oxidant | 0.35 | 0.39 |
| (A) | Base Oil | Balance | Balance |
| | | | |
| | TBN | 7.1 | 8 |
| | Ash (sulfated) (%) | 0.45 | 0.50 |
| (Antifoams were also present) | | | |

The above figures, where appropriate, represent mass % of an additive components that, with the exception of (F), includes diluent or solvent. The figure for (F) represents active ingredient.

### Comparison Examples

As comparison gas-fuelled engine lubricating oil compositions (Examples A and B), there were used commercially available lubricating oils, the detergency of each of which was phenate-based and was salicylate-free. Example A had a TBN of 5.2 and 0.45% sulfated ash and Example B had a TBN of 8.8 and 0.80% sulfated ash.

### TESTS

Samples of Examples 1, 2, A and B were each tested according to the GFC T-021-A-90 procedure, an industry standard, at 170°C for a period of 216 hours, with an intermediate sampling after 144 hours.

The samples were analysed for:
- kinematic viscosity at 100°C (ASTM D445)
- TAN (ASTM D664)
- TBN (ASTM D2896)
- Infra-Red Oxidation and Nitration (spectroscopic method known in the art)

The identity of the method is indicated in parentheses

### RESULTS

The results of the tests are summarised in the table below.

| SAMPLE | TEST | TEST TIME (hours) | | |
|---|---|---|---|---|
| (EXAMPLE REF) | | 0 | 144 | 216 |
| 1 | VISCOSITY | 14.08 | 15.43 | 17.43 |
| 2 | (mm²s⁻¹) | 14.38 | 15.37 | 17.59 |
| A | | 13.66 | 23.27 | - |
| B | | 14.05 | 18.25 | 26.89 |
| 1 | TAN | 0.59 | 2.02 | 4.14 |
| 2 | (mg KOHg⁻¹) | 0.65 | 0.71 | 3.65 |
| A | | 0.44 | 5.64 | 8.22 |
| B | | 0.38 | 4.45 | 7.17 |
| 1 | TBN | 7.12 | 2.47 | 1.44 |
| 2 | (mg KOHg⁻¹) | 7.96 | 3.08 | 1.75 |
| A | | 5.22 | 0.5 | 0.5 |
| B | . | 8.81 | 0.5 | 0.5 |
| 1 | IR Oxidation | 0 | 28.91 | 54.69 |
| 2 | (cm⁻¹) | 0 | 25.00 | 50.78 |
| A | | 0 | 54.41 | - |
| B | | 0 | 47.06 | 70.59 |
| 1 | IR Nitration | 0 | 3.13 | 7.81 |
| 2 | (cm⁻¹) | 0 | 3.13 | 6.25 |
| A | | 0 | 20.59 | - |
| B | | 0 | 12.50 | 22.79 |

A dash indicates that the sample was too thick to measure. In all tests (apart from TBN), lower values indicate superior performance. Thus, the results show the superiority of Examples 1 and 2 over each of Examples A and B that lacked salicylate.

## Claims

1. A gas-fuelled engine lubricating oil composition having a TBN in the range of 2 to 20 comprising:
(A) an oil of lubricating viscosity, in a major amount; and added thereto, in respective minor amounts:
(B) one or more metal hydrocarbyl-substituted salicylate detergents having a TBN of 95 or less;
(C) one or more calcium salicylate, phenate or complex detergents having a TBN of greater than 250;
(D) one or more dispersants, such as an ashless dispersant; and
(E) preferably one or more anti-wear additives.

2. The composition as claimed in claim 1, further added thereto, in a minor amount, being (F) one or more antioxidants, such as amine or phenolic anti-oxidants.

3. The composition as claimed in claim 1 or claim 2, wherein the metal of the hydrocarbyl-substituted salicylate (B) is calcium.

4. The composition as claimed in any of claims 1 to 3, wherein the calcium detergent (C) is a calcium hydrocarbyl-substituted salicylate or a calcium complex detergent that contains a salicylate surfactant, having a TBN in the range of 250 to 500, preferably 260 to 400.

5. The composition as claimed in any of claims 2 to 4, wherein the anti-oxidant (F) is present in the composition in an amount of up to 3 mass %.

6. A method of lubricating a gas-fuelled internal combustion engine comprising operating the engine and lubricating it with a composition as claimed in any of claims 1 to 5.

7. A method for enhancing the resistance of a gas-fuelled lubricating oil composition to oxidation and nitration, the method comprising the step of adding the composition with additives (B) to (F) as defined in any of claims 1 to 5 to the gas-fuelled engine lubricating oil composition.

8. An additive package or concentrate for a gas-fuelled engine lubricating oil composition, comprising:
(B) one or more metal hydrocarbyl-substituted salicylate detergents having a TBN of 95 or less;
(C) one or more calcium salicylate, phenate or complex detergents having a TBN of greater than 250;
(D) one or more dispersants, such as an ashless dispersant; and
(E) preferably one or more anti-wear additives.

## Patentansprüche

1. Schmierölzusammensetzung für einen gasbetriebenen Motor mit einer TBN im Bereich von 2 bis 20, die:
(A) in einer größeren Menge Öl von Schmierviskosität und dazu hinzugefügt jeweils in kleineren Mengen:
(B) ein oder mehrere mit Kohlenwasserstoffrest substituierte Metallsalicylatdetergenzien mit einer TBN von 95 oder weniger,
(C) ein oder mehrere Calciumsalicylat-, Phenat- oder Komplexdetergenzien mit einer TBN von größer als 250,
(D) ein oder mehrere Dispergiermittel, wie ein aschefreies Dispergiermittel, und
(E) vorzugsweise ein oder mehrere Antiverschleißadditive umfasst.

2. Zusammensetzung nach Anspruch 1, der ferner in einer kleineren Menge als (F) ein oder mehrere Antioxidanzien, wie Amin oder phenolische Antioxidanzien, zugesetzt sind.

3. Zusammensetzung nach Anspruch 1 oder Anspruch 2, wobei das Metall des mit Kohlenwasserstoffrest substituierten Salicylats (B) Calcium ist.

4. Zusammensetzung nach einem der Ansprüche 1 bis 3, wobei das Calciumdetergens (C) ein mit Kohlenwasserstoffrest substituiertes Calciumsalicylat oder ein Calciumkomplexdetergens ist, das ein Salicylattensid mit einer TBN im Bereich von 250 bis 500, vorzugsweise 260 bis 400 enthält.

5. Zusammensetzung nach einem der Ansprüche 2 bis 4, wobei das Antioxidanz (F) in der Zusammensetzung in einer Menge von bis zu 3 Masse-% vorliegt.

6. Verfahren zum Schmieren eines mit Gas betriebenen Verbrennungsmotors, bei dem der Motor betrieben wird und er mit einer Zusammensetzung gemäß einem der Ansprüche 1 bis 5 geschmiert wird.

7. Verfahren zur Erhöhung der Widerstandsfähigkeit einer Schmierölzusammensetzung für einen mit Gas betriebenen Motor gegenüber Oxidation und Nitrierung, bei dem die Zusammensetzung mit den Additiven (B) bis (F) wie in einem der Ansprüche 1 bis 5 definiert zu der Schmierölzusammensetzung für den mit Gas betriebenen Motor gegeben wird.

8. Additivpaket oder -konzentrat für eine Schmierölzusammensetzung für einen mit Gas betriebenen Motor, das:
(B) ein oder mehrere mit Kohlenwasserstoffrest substituierte Metallsalicylatdetergenzien mit einer TBN von 95 oder weniger,
(C) ein oder mehrere Calciumsalicylat-, Phenat- oder Komplexdetergenzien mit einer TBN von größer als 250,
(D) ein oder mehrere Dispergiermittel, wie ein aschefreies Dispergiermittel, und
(E) vorzugsweise ein oder mehrere Antiverschleißadditive umfasst.

## Revendications

1. Composition d'huile lubrifiante pour moteur à alimentation au gaz ayant un indice de basicité totale (IBT) dans la gamme de 2 à 20 comprenant :
(A) une huile de viscosité de lubrification, en une quantité majoritaire ; et, ajoutés à celle-ci, en quantités minoritaires respectives :
(B) un ou plusieurs détergents de type salicylate de métal substitué par un groupe hydrocarbyle ayant un IBT inférieur ou égal à 95 ;
(C) un ou plusieurs détergents de type complexe, phénate ou salicylate de calcium ayant un IBT supérieur à 250 ;
(D) un ou plusieurs dispersants, tels qu'un dispersant sans cendre ; et
(E) de préférence un ou plusieurs additifs anti-usure.

2. Composition selon la revendication 1, à laquelle on a ajouté en outre, en une quantité minoritaire, (F) un ou plusieurs antioxydants, tels que des antioxydants de type amine ou phénolique.

3. Composition selon la revendication 1 ou la revendication 2, dans laquelle le métal du salicylate substitué par un groupe hydrocarbyle (B) est le calcium.

4. Composition selon l'une quelconque des revendications 1 à 3, dans laquelle le détergent à base de calcium (C) est un salicylate de calcium substitué par un groupe hydrocarbyle ou un détergent de type complexe de calcium qui contient un agent tensioactif de type salicylate, ayant un IBT dans la gamme de 250 à 500, de préférence de 260 à 400.

5. Composition selon l'une quelconque des revendications 2 à 4, dans laquelle l'antioxydant (F) est présent dans la composition en une quantité allant jusqu'à 3 % en masse.

6. Procédé de lubrification d'un moteur à combustion interne à alimentation au gaz comprenant le fait de faire fonctionner le moteur et de le lubrifier avec une composition selon l'une quelconque des revendications 1 à 5.

7. Procédé destiné à augmenter la résistance à l'oxydation et à la nitration d'une composition d'huile de lubrification pour moteur à alimentation au gaz, le procédé comprenant l'étape consistant à ajouter la composition avec les additifs (B) à (F) telle que définie selon l'une quelconque des revendications 1 à 5 à la composition d'huile de lubrification pour moteur à alimentation au gaz.

8. Ensemble ou concentré d'additifs pour une composition d'huile de lubrification pour moteur à alimentation au gaz, comprenant :
(B) un ou plusieurs détergents de type salicylate de métal substitué par un groupe hydrocarbyle ayant un IBT inférieur ou égal à 95 ;
(C) un ou plusieurs détergents de type complexe, phénate ou salicylate de calcium ayant un IBT supérieur à 250 ;
(D) un ou plusieurs dispersants, tels qu'un dispersant sans cendre ; et
(E) de préférence un ou plusieurs additifs anti-usure.
